

[54] GREASE THICKENED WITH  
OXYGEN-LINKED POLYUREAS

[75] Inventor: **Eberhard Gegner**, Hamburg,  
Germany

[73] Assignee: **The British Petroleum Company  
Limited**, London, England

[22] Filed: **Nov. 29, 1973**

[21] Appl. No.: **420,004**

[30] Foreign Application Priority Data

Dec. 11, 1972 Germany ..... 2260496

[52] U.S. Cl. ..... 252/51.5 A, 252/403

[51] Int. Cl. .... C10m 5/20, C10m 7/32, C10m 7/30

[58] Field of Search ..... 252/51.5 A, 403

[56] References Cited

UNITED STATES PATENTS

|           |        |                       |            |
|-----------|--------|-----------------------|------------|
| 3,243,372 | 3/1966 | Dreher et al. ....    | 252/51.5 A |
| 3,374,170 | 3/1968 | Hedenburg et al. .... | 252/51.5 A |
| 3,725,279 | 4/1973 | Armstrong ....        | 252/51.5 A |

Primary Examiner—Delbert E. Gantz  
Assistant Examiner—I. Vaughn

[57] ABSTRACT

Grease thickened with oxygen-linked polyureas.

31 Claims, No Drawings

## GREASE THICKENED WITH OXYGEN-LINKED POLYUREAS

This invention relates to a process for the production of novel polyureas and to a process for the production of greases thickened by such polyureas.

Greases containing polyureas as thickeners have been disclosed. Thus, for example U.S. Pat. No. 3243372 describes greases containing polyureas of general formula



in which  $R^1$  and  $R^{111}$  represent monovalent and  $R$  and  $R^{111}$  represent divalent hydrocarbon radicals and  $X$  is an integer from 1 to 3.

Greases in accordance with U.S. Pat. No. 3 243 372 are produced by dissolving a di-isocyanate in the lubricating oil which is to be thickened, optionally by making use of a further solvent, adding amines to this mixture and then heating the total mixture, the polyurea being formed in situ.

Greases with polyureas as thickeners are chemically resistant to water and oxidation; they decompose under the action of heat only at relatively high temperatures.

Our copending British Pat. application No. 2774/73 corresponding to U.S. Pat. application Ser. No. 329,686 filed Feb. 5, 1973, discloses that diamines containing sulphur and mixtures of aliphatic and aromatic mono-amines may be used as the amine components for the production of polyureas in lubricating oils.

Greases thickened with such polyureas are distinguished by improved mechanical stability and increased load-bearing capacity.

It has now surprisingly been found that greases with still further improved properties are obtained if the polyureas used as thickeners and produced in situ from a mono-amino, a diamino and a di-isocyanate component contain in their chains oxygen bridges as structural elements, and are partially asymmetrical in relation to the nature of the terminal groups.

Greases with such polyureas as thickeners are chemically resistant to water, oxidation and the action of heat; they also possess good load-bearing capacity and mechanical stability. Furthermore they are distinguished by a reduced tendency to gel or harden.

The last mentioned property is of great importance for the satisfactory lubrication of bearings. Gelling or hardening caused by purely thermal influences is caused by a structural alteration in a grease. It is true that this alteration can sometimes be reversed by mechanical stress. If portions of grease, however, occur in a bearing subject to great thermal stress outside the ranges of mechanical stress, and should these portions then gel or harden as mentioned, there is a risk that insufficient grease may be supplied for lubrication. This can cause dry running and hence the destruction of the bearing concerned. This risk is considerably reduced, however, for bearings which are lubricated with a grease according to the invention.

Thus according to the present invention there is provided a process for the production of a polyurea which process comprises reacting a monoamino, a diamino and a di-isocyanate component at a temperature in the range 20° to 150°C wherein

a. the monoamino component comprises a mixture of at least two members selected from different groups of general formulae:



5 in which  $R^1$  is a monovalent aliphatic radical containing 12 to 24 carbon atoms,  $R_2$  is a monovalent aromatic radical,  $R^3$  is a monovalent aliphatic radical containing 2 to 10 carbon atoms and  $R^4$  is a divalent aliphatic radical containing 2 to 4 carbon atoms.

b. the diamino component comprises a dioxo-alkane diamine or a mixture of dioxo-alkanediamines of general formula:



15 in which  $R^5$  and  $R^7$  are divalent aliphatic radicals containing 2 to 4 carbon atoms and  $R^6$  is a divalent aliphatic radical containing 2 to 10 carbon atoms, and

c. the di-isocyanate component comprises an aromatic di-isocyanate or a mixture of aromatic diisocyanates.

According to a further feature of the invention there is provided a process for the production of a grease which process comprises reacting a monoamino, a diamino and a di-isocyanate component in a lubricating oil at a temperature in the range 20° to 150°C wherein (a) the monoamino component comprises a mixture of at least two members selected from different groups of general formulae:



35 in which  $R^1$  is a monovalent aliphatic radical containing 12 to 24 carbon atoms,  $R^2$  is a monovalent aromatic radical,  $R^3$  is a monovalent aliphatic radical containing 2 to 10 carbon atoms and  $R^4$  is a divalent aliphatic radical containing 2 to 4 carbon atoms.

40 b. the diamino component comprises a dioxo-alkanediamine or a mixture of dioxo-alkanediamines of general formula:



45 in which  $R^5$  and  $R^7$  are divalent aliphatic radicals containing 2 to 4 carbon atoms, and  $R^6$  is a divalent aliphatic radical containing 2 to 10 carbon atoms, and

50 c. the di-isocyanate component comprises an aromatic di-isocyanate or a mixture of aromatic diisocyanates. The components are preferably reacted at a temperature of in the range 40° to 70°C.

If desired the reaction mixture is then heated further to a temperature of 150° to 200°C, preferably to about 175°C. By this treatment under controlled conditions an additional improvement of the properties of the greases of the invention is achieved, which presumably can be attributed to trans-amidation and cross-linking reactions in the polyureas.

According to a further advantageous feature of the invention the di-isocyanate component, optionally at a temperature which is above its melting point, or dissolved in lubricating oil or in a solvent which is inert under the reaction conditions, is added to the mixture of mono-amino and diamino components and the lubricating oil. The di-isocyanate component is thus exposed during the reaction to an excess of amines, as a result of which the degree of branching or cross-linking

of the polyureas in the grease can be controlled in an advantageous manner.

The molar ratio between mono-amino component, diamino component and di-isocyanate component preferably lies in the range from 2:1:2 to 2:1:2.5 or in the range from 2:2:3 to 2:2:3.75 when with a stoichiometrical excess of di-isocyanate component, cross-linkings or branchings of the polyurea chains additionally occur. As a result of this the advantageous properties of the greases of the invention can be further improved.

When using an aliphatic mono-amine or several aliphatic mono-amines and an aromatic mono-amine or several aromatic mono-amines as mono-amino component, the compounds corresponding to the formulae given previously, the molar ratio of aliphatic mono-amine or mono-amines to aromatic mono-amine or mono-amines is preferably about 1:1.

When using an aliphatic mono-amine or several aliphatic mono-amines and an aliphatic mono-amino-ether or several aliphatic mono-amino-ethers as mono-amino component, the compounds corresponding to the formulae given previously the molar ratio of aliphatic mono-amine or mono-amines to aliphatic mono-amino-ether or aliphatic mono-amino-ethers is preferably about 1:1.

When using an aromatic mono-amine or several aromatic mono-amines and an aliphatic mono-amino-ether or several aliphatic mono-amino-ethers as mono-amino component, the compounds corresponding to the formulae given previously, the molar ratio of aromatic mono-amine or mono-amines to aliphatic mono-amino-ether or aliphatic mono-amino-ethers is preferably about 1:1.

When using an aliphatic mono-amine or several aliphatic mono-amines and an aromatic mono-amine or several aromatic mono-amines and an aliphatic mono-amino-ether or several aliphatic mono-amino-ethers as mono-amino component, the compounds corresponding to the formulae given previously, the molar ratio of aliphatic mono-amine or mono-amines to aromatic mono-amines or mono-amines to aliphatic mono-amino-ether or aliphatic mono-amino-ethers is preferably about 1:0.5:0.5.

For the production of polyureas according to the invention the aliphatic mono-amine in the mono-amino component is preferably a straight-chained mono-amine with 16 to 24 carbon atoms per molecule, or a mixture of such mono-amines.

The aromatic mono-amine in the mono-amino component is preferably aniline, toluidine or xylidine or a mixture of these amines. Isomeric aromatic mono-amines can be used individually or as an isomer mixture.

The aliphatic mono-amino-ether of the general formula



is preferably one in which  $R^3$  is a monovalent aliphatic radical containing 4 to 6 carbon atoms and  $R^4$  is a divalent aliphatic radical containing 2 or 3 carbon atoms. These mono-amino-ethers can be used separately or as mixtures.

The dioxa-alkanediamine of the general formula



is preferably one in which  $R^5$  and  $R^7$  are divalent ali-

phatic radicals containing 2 or 3 carbon atoms and  $R^6$  is a divalent aliphatic radical containing 4 to 6 carbon atoms. The dioxa-alkanediamine can be used singly or as a mixture.

Preferred aromatic di-isocyanates include phenylene, toluylene, ditoluylene, naphthylene or diphenylene methane di-isocyanate or mixtures thereof. Isomeric di-isocyanates can be used singly or as isomer mixtures.

In a suitable manner after cooling to about 100°C

10 conventional grease additives can be added, for example to improve boundary lubrication properties, resistance to oxidation, corrosion protection and the like.

After cooling, grease obtained by the process described above may be homogenised by conventional methods, e.g., colloid milling.

Prior to homogenising a further quantity of lubricating oil can be added if initially a higher concentration of thickener has been produced in the reaction mixture than is later desired in the finished grease.

20 Suitably the concentration of thickener in a grease according to the invention is in the range from 3 to 30% by weight.

Any usual lubricating oil can be thickened. For example, paraffin-based or naphthene-based lubricating

25 oil fractions or mixtures of such fractions are suitable. Synthetic lubricating oils such as polyarylene ethers, polyalkylene glycols, polysiloxanes or ester oils which are obtained (for example) by reacting monobasic and/or

30 polybasic carboxylic acids with monohydric and/or polyhydric alcohols, may also be used for the production of the greases.

The invention is illustrated with reference to the following Examples.

### EXAMPLE 1

35 A mixture of 42.2 g of 4,9-dioxadodecane-1,12-diamine, 63.6 g Genamin 20/22 R 100 D (mixture of primary amines with chain lengths of  $C_{18}$ ,  $C_{20}$  and  $C_{24}$  in the ratio 4:39:54:3), 22.2 g p-toluidine and 1,500 g

40 of a mixed-base solvent raffinate (14°E/50°C corresponding to 105 cSt/50°C) was heated to 60°C with stirring. At this temperature the amines dissolved in the mineral oil to form a clear solution. With constant intensive stirring 72.0 g. of Desmodur T 65 (mixture of

45 65% 2,4-tolylene di-isocyanate and 35% 2,6-toluylene diisocyanate) was added dropwise over a period of 10 minutes. The turbidity which immediately set in increased rapidly, and the contents of the reactor thickened. For rinsing, a further 100 g of the same base oil

50 was added to the feed vessel for the di-isocyanates. The reaction mixture was then heated with further stirring to 175°C, and when this temperature was reached the mixture was cooled to 100°C. A mixture of 10 g of

55 Amine T (corrosion inhibitor by Ciba-Geigy), 20 g Adititin 30 (oxidation inhibitor by Farbenfabriken Bayer), 2 g Reomet SBT (metal de-activator by Ciba-Geigy) and 168 g base oil were then added and the mixture stirred until cold. When cold the grease was homogenised in a colloid mill.

60 The molar ratio of the reaction components (mono-amine 1: mono-amine 2:4,9-dioxadodecane-1, 12-diamine:di-isocyanate) was 1:1:1:2.

|                                         |       |
|-----------------------------------------|-------|
| Thickener content of lubricant grease   | 10%   |
| Drop point (DIN 51 801, Sheet 1)        | 220°C |
| Worked penetration (DIN 51 804 Sheet 2) | 287   |

-Continued

|                                                                                   |             |
|-----------------------------------------------------------------------------------|-------------|
| Corrosion index according to Emcor Test (DIN 51 802)                              | 0           |
| Oil separation (IP 121/63)                                                        | 1.3% by wt. |
| Mechanical/Dynamic SKF test (DIN 51 806):<br>A run (2,500 r.p.m. without heating) | passed      |
| B run (1,500 r.p.m., 130°C)                                                       | passed      |

## EXAMPLE 2

A mixture of 41.5 g. of 4,9-dioxadodecane-1,12-diamine, 62.4 g of Genamin 20/22 R 100 D, 21.8 g of p-toluidine and 1,500 g of a mixed-base solvent raffinate (14°C/50°C corresponding to 105 cSt/50°C) was heated to 60°C with stirring. The amines formed a clear solution with the mineral oil at this temperature. Maintaining constant stirring, 74.3 g of Desmodur T 65 were added dropwise over 10 minutes. The turbidity which immediately set in increased rapidly, and the contents of the reactor thickened. For rinsing, a further 100 g of the same base oil were added to the feed vessel for the di-isocyanates. The reaction mixture was then heated with further stirring to 175°C, and after reaching this temperature the mixture was cooled to 100°C. A mixture of 10 g of Amine T, 20 g of Additin 30, 2 g of Reomet SBT and 168 of base oil was then added, and the mixture stirred until cold. When cold the grease was homogenised in a colloid mill.

The molar ratio of the reaction components (mono-amine 1: monoamine 2:4,9-dioxadodecane-1,12-diamine:di-isocyanate was 1:1:1:2.1.

|                                                                                   |             |
|-----------------------------------------------------------------------------------|-------------|
| Thickener content of the lubricant grease                                         | 10%         |
| Drop point (DIN 51 801, Sheet 1)                                                  | 244°C       |
| Worked penetration (DIN 51 804, Sheet 2)                                          | 305         |
| Corrosion index according to Emcor Test (DIN 51 802)                              | 0           |
| Oil separation (IP 121/63)                                                        | 1.6% by wt. |
| Mechanical/Dynamic SKF test (DIN 51 806):<br>A run (2,500 r.p.m. without heating) | passed      |
| B run (1,500 r.p.m. at 130°C)                                                     | passed      |

## EXAMPLE 3

A mixture of 41.2 g of 4,9-dioxadodecane-1,12-diamine, 62.0 g of Genamin 20/22 R 100 D, 26.5 g of butoxypropylamine and 1,500 g of a mixed-base solvent raffinate (14°C/50°C corresponding to 105 cSt/50°C) was heated to 60°C with stirring. The amines formed a clear solution with the mineral oil at this temperature. With constant intensive stirring 70.3 g of Desmodur T 65 was added dropwise over 10 minutes. The turbidity which immediately set in increased rapidly, and the contents of the reactor thickened. For rinsing, a further 100 g of the same base oil were added to the feed vessel for the di-isocyanates. The reaction mixture was then heated with further stirring to 175°C. When this temperature was reached the mixture was cooled to 100°C, and a mixture of 10 g of Amine T, 20 g of Additin 30, 2 g of Reomet SBT and 168 g of base oil was then added. The mixture was then stirred until cold. When cold the grease was homogenised in a colloid mill.

The molar ratio of the reaction components mono-amine 1: mono-amine 2: 4,9-dioxadodecane-1,12-diamine:di-isocyanate was 1:1:1:2.

|                                                                                   |             |
|-----------------------------------------------------------------------------------|-------------|
| Thickener content of the grease                                                   | 10%         |
| Drop point (DIN 51 801, Sheet 1)                                                  | 203°C       |
| Worked penetration (DIN 51 804 Sheet 2)                                           | 268         |
| Corrosion index according to Emcor Test (DIN 51 802)                              | 0           |
| Oil separation (IP 121/63)                                                        | 2.1% by wt. |
| Mechanical/Dynamic SKF test (DIN 51 806):<br>A run (2,500 r.p.m. without heating) | passed      |
| B run (1,500 r.p.m. at 130°C)                                                     | passed      |

10

## EXAMPLE 4

A mixture of 40.1 g of 4,9-dioxadodecane-1,12-diamine, 60.3 g of Genamin 20/22 R 100 D, 31.2 g of hexyloxy-propylamine and 1,500 g of a mixed-base solvent raffinate (14°C/50°C corresponding to 105 cSt/50°C) was heated to 60°C with stirring. The amines formed a clear solution with the mineral oil at this temperature. Maintaining constant intensive stirring, 68.4 g of Desmodur T 65 were added dropwise over 10 minutes. The turbidity which set in immediately increased rapidly and the contents of the reactor thickened. For rinsing a further 100 g of the same base oil were added to the feed vessel for the di-isocyanates. The reaction mixture was then heated with further stirring to 175°C. After reaching this temperature the mixture was cooled to 100°C and a mixture of 10 g of Amine T, 20 g of Additin 30, 2 g of Reomet SBT and 168 g of base oil were then added. The mixture was then stirred until cold. When cold the lubricant grease was homogenised in a colloid mill.

The molar ratio of the reaction components (mono-amine 1: monoamine 2:4,9-dioxadodecane-1,12-diamine:di-isocyanate) was 1:1:1:2.

|                                                                                   |             |
|-----------------------------------------------------------------------------------|-------------|
| Thickener content of the lubricant grease                                         | 10%         |
| Drop point (DIN 51 801, Sheet 1)                                                  | 205°C       |
| Worked penetration (DIN 51 804, Sheet 2)                                          | 265         |
| Corrosion index according to Emcor Test (DIN 51 802)                              | 0           |
| Oil separation (IP 121/63)                                                        | 1.7% by wt. |
| Mechanical/Dynamic SKF test (DIN 51 806):<br>A run (2,500 r.p.m. without heating) | passed      |
| B run (1,500 r.p.m. at 130°C)                                                     | passed      |

45

I claim:

1. A process for the production of a grease which process comprises reacting a monoamino, a diamino and a di-isocyanate component in a lubricating oil at a temperature in the range 20° to 150°C wherein

50 a. the monoamino component comprises a mixture of at least two members selected from different groups of general formulae:



60 in which  $R^1$  is a monovalent aliphatic radical containing 12 to 24 carbon atoms,  $R^2$  is a monovalent aromatic radical,  $R^3$  is a monovalent aliphatic radical containing 2 to 10 carbon atoms and  $R^4$  is a divalent aliphatic radical containing 2 to 4 carbon atoms,

65 b. the diamino component comprises a dioxoalkanediamine or a mixture of dioxoalkanediamines of general formula:



in which  $\text{R}^5$  and  $\text{R}^7$  are divalent aliphatic radicals containing 2 to 4 carbon atoms, and  $\text{R}^6$  is a divalent aliphatic radical containing 2 to 10 carbon atoms, and

c. the di-isocyanate component comprises an aromatic di-isocyanate or a mixture of aromatic di-isocyanates wherein the molar ratio between monoamino, diamino and di-isocyanate components is in the range of 2:1:2 to 2:2:3.75.

2. A process according to claim 1 wherein the reaction is carried out at a temperature in the range 40° to 70°C.

3. A process according to claim 1 wherein the reaction mixture is subsequently heated to a temperature in the range 150° to 200°C.

4. A process according to claim 1 wherein the di-isocyanate component is added to a mixture of the monoamino and diamino components.

5. A process according to claim 4 wherein the di-isocyanate component is added in molten form or dissolved in a lubricating oil or an inert solvent.

6. A process according to claim 1 wherein the molar ratio between monoamino, diamino and di-isocyanate components is in the range 2:1:2 to 2:1:2.5.

7. A process according to claim 1 wherein the molar ratio between monoamino, diamino and di-isocyanate compounds is in the range 2:2:3 to 2:2:3.75.

8. A process according to claim 1 wherein two monoamino compounds are present in a molar ratio of 1:1.

9. A process according to claim 1 wherein three monoamino compounds are present in a molar ratio of 1:0.5:0.5.

10. A process according to claim 1 wherein the monoamino component comprises a monoamine of general formula  $\text{R}^1-\text{NH}_2$  in which  $\text{R}^1$  is a monovalent aliphatic radical containing 16 to 24 carbon atoms.

11. A process according to claim 1 wherein the monoamino component comprises an aromatic monoamine which is aniline, toluidine, xylidine, or a mixture thereof.

12. A process according to claim 1 wherein the monoamino component comprises a monoamine of general formula  $\text{R}^3-\text{O}-\text{R}^4-\text{NH}_2$  in which  $\text{R}^3$  is a monovalent aliphatic radical containing 4 to 6 carbon atoms and  $\text{R}^4$  is a divalent aliphatic radical containing 1 or 3 carbon atoms.

13. A process according to claim 1 wherein the diamino component comprises a straight chain dioxo-alkane diamine of general formula  $\text{NH}_2-\text{R}^5-\text{O}-\text{R}^6-\text{O}-\text{R}^7-\text{NH}_2$  in which  $\text{R}^5$  and  $\text{R}^7$  are divalent aliphatic radicals containing 2 or 3 carbon atoms and  $\text{R}^6$  is a divalent aliphatic radical containing 4 to 6 carbon atoms.

14. A process according to claim 1 wherein the di-isocyanate component comprises phenylene, tolylene-, ditolylene-, naphthylene, or diphenylmethane di-isocyanate, or mixtures thereof.

15. A process according to claim 1 wherein the lubricating oil is a mineral oil, a polyaryl ether, a polyalkylene glycol, a polysiloxane or an ester.

16. A process according to claim 15 wherein the mineral lubricating oil is a paraffinic or naphthenic lubricating oil fraction or a mixture thereof.

17. A process according to claim 1 wherein the grease contains 3 to 30% by weight of the polyurea.

18. A grease composition comprising a lubricating oil thickened by 3-30% by weight of a polyurea formed in situ, said composition being formed by a process which comprises reacting a monoamino component and a diamino component with a di-isocyanate component in a lubricating oil at a temperature in the range 20° to 150°C wherein

10 a. the monoamino component comprises a mixture of at least two members selected from the following general formulae:



15 in which  $\text{R}^1$  is a monovalent aliphatic radical containing 12 to 24 carbon atoms,  $\text{R}^2$  is a monovalent aromatic radical,  $\text{R}^3$  is a monovalent aliphatic radical containing 2 to 10 carbon atoms and  $\text{R}^4$  is a divalent aliphatic radical containing 2 to 4 carbon atoms,

20 b. the diamino component comprises a dioxo-alkane diamine or a mixture of dioxo-alkanediamines of the general formula:  $\text{NH}_2-\text{R}^5-\text{O}-\text{R}^6-\text{O}-\text{R}^7-\text{NH}_2$

25 in which  $\text{R}^5$  and  $\text{R}^7$  are divalent aliphatic radicals containing 2 to 4 carbon atoms and  $\text{R}^6$  is a divalent aliphatic radical containing 2 to 10 carbon atoms, and

30 c. the di-isocyanate component comprises an aromatic di-isocyanate or a mixture of aromatic di-isocyanates wherein the molar ratio of the monoamino, diamino and di-isocyanate components is in the range of 2:1:2 to 2:2:3.75.

35 19. The composition of claim 18 wherein the molar ratio between monoamino, diamino and di-isocyanate components is in the range 2:1:2 to 2:1:2.5.

20. The composition of claim 18 wherein the molar ratio between monoamino, diamino and di-isocyanate components is in the range 2:2:3.75.

40 21. The composition of claim 18 wherein two monoamino compounds are present in a molar ratio of 1:1.

45 22. The composition of claim 18 wherein three monoamino compounds are present in a molar ratio of 1:0.5:0.5.

50 23. The composition of claim 18 wherein the monoamino component comprises a monoamine of the general formula  $\text{R}^1-\text{NH}_2$  in which  $\text{R}^1$  is a monovalent aliphatic radical containing 16 to 24 carbon atoms.

55 24. The composition of claim 18 wherein the monoamino component comprises an aromatic monoamine which is aniline, toluidine, xylidine, or a mixture thereof.

60 25. The composition of claim 18 wherein the monoamino component comprises a monoamine of the general formula  $\text{R}^3-\text{O}-\text{R}^4-\text{NH}_2$  in which  $\text{R}^3$  is a monovalent aliphatic radical containing 4 to 6 carbon atoms and  $\text{R}^4$  is a divalent aliphatic radical containing 2 or 3 carbon atoms.

65 26. The composition of claim 18 wherein the diamino component comprises a straight chain dioxo-alkane diamine of the general formula  $\text{NH}_2-\text{R}^5-\text{O}-\text{R}^6-\text{O}-\text{R}^7-\text{NH}_2$  in which  $\text{R}^5$  and  $\text{R}^7$  are divalent aliphatic radicals containing 2 or 3 carbon atoms and  $\text{R}^6$  is a divalent aliphatic radical containing 4 to 6 carbon atoms.

27. The composition of claim 18 wherein the diisocyanate component comprises phenylene, toluylene-, ditolylene-, naphthylene, or diphenylmethane diisocyanate, or mixtures thereof.

28. The composition of claim 18 wherein the lubricating oil is a mineral oil, a polyaryl ether, a polyalkylene glycol, a polysiloxane or an ester.

29. The composition of claim 28 wherein the mineral lubricating oil is a paraffinic or naphthenic lubricating

oil fraction or a mixture thereof.

30. The composition of claim 18 wherein the reaction is carried out at a temperature in the range 40° to 70°C.

31. The composition of claim 18 wherein the reaction mixture is subsequently heated to a temperature in the range 150° to 200°C.

\* \* \* \* \*

UNITED STATES PATENT AND TRADEMARK OFFICE  
CERTIFICATE OF CORRECTION

PATENT NO. : 3,870,642  
DATED : March 11, 1975  
INVENTOR(S) : Eberhard Gegner

It is certified that error appears in the above-identified patent and that said Letters Patent are hereby corrected as shown below:

Column 1, line 10, "NH—CO—NHR<sup>111</sup>" should be --NH—CO—NHR<sup>111</sup>--; line 11, "—<sub>x</sub> CO" should be --  $\frac{1}{x}$  CO --. Column 3, line 29, "mon-amino" should be --mono-amino--; line 42, "mono-amines or mono-amines" should be --mono-amine or mono-amines--; line 66, "—O—R<sup>7</sup>—" should be -- —O—R<sup>7</sup>— --. Column 4, line 41, Column 5, line 49 and Column 6, line 17, "14°E/50°C", each occurrence, should read --14°C/50°C--. Column 4, line 29, "plybasic" should be --polybasic--; line 47, "dioisocyanate" should be --di-isocyanate--; line 68, "DINN" should be --DIN--. Column 5, line 40, "DIn" should be --DIN--; line 67, "dioxaodecane" should be --dioxadodecane--. Column 6, line 40, "265" should be moved to right column of chart. Column 7, line 4, "divia—" should be --diva- --; line 49, the number "1" should be --2--.

Signed and Sealed this

thirtieth Day of September 1975

[SEAL]

Attest:

RUTH C. MASON  
Attesting Officer

C. MARSHALL DANN  
Commissioner of Patents and Trademarks